

## UNITED STATES PATENT OFFICE.

LESTER KIRSCHBRAUN, OF CHICAGO, ILLINOIS.

## EMULSIFIED FUEL.

No Drawing. Application filed April 5, 1920, Serial No. 371,258. Renewed July 5, 1928.

This invention relates to emulsified hydrocarbon fuels and to a new and improved fuel and the method of making such fuels. Among the objects are to produce a fuel of 5 the character mentioned which will have great stability and can be economically made and which will be effective in use, both from the standpoint of power developed and the elimination of carbon deposits in the 10 engine. The invention also contemplates the forming of a primary emulsion and then forming a second emulsion or in some cases diluting the first emulsion with a different hydrocarbon oil.

15 Describing first that form of the invention in which one emulsion itself forms the dispersed or internal phase of the final product, the process is as follows: A given percent of water, for example, an amount of water 20 equal to 10 percent of the final product, is mixed with a small percentage, for example, one percent of a water soluble oil or other soap or suitable emulsifying agent and the water and emulsifying agent is then mixed 25 with a hydrocarbon oil, for example, an amount of gasoline equal to 10 percent of the final product. This mixture is preferably run through a homogenizer giving a white colored product which is an emulsion 30 having the water in the continuous phase. The product thus far obtained is then used as the dispersed phase and dispersed in a hydrocarbon oil preferably a hydrocarbon oil containing about one percent of an oil 35 soluble emulsifying agent. Such an agent has been employed which was a petroleum itself—this being a naphthenic acid or a sulphonic derivative of naphthenic hydrocarbon. The resultant emulsion also if desired can be run through the homogenizer 40 and the final product employed in the ordinary internal combustion engine in place of the usual gasoline.

In place of forming the double emulsion, 45 the process may be varied so as to first produce an emulsion of water with a heavy hydrocarbon oil, the oil in this case being in the continuous phase with the water very finely dispersed therein. This initial product is preferably run through a homogenizer 50 and then diluted with gasoline or other

desired hydrocarbon oil, and as the emulsifying agent in this case is oil soluble the initial emulsion will not be broken by the addition of more hydrocarbon oil. Both of 55 the processes contemplate an initial emulsion and the addition of a greater amount of oil, but both methods mentioned as well as the resultant products can be varied without departing from the scope of the 60 invention set forth in the claims.

It will be understood that one of the advantages of using the relatively heavy hydrocarbon oil in the primary emulsion is to derive the advantages of greater dispersion 65 which will be effective on account of the greater viscosity of oil of this character. Also the stability of the final emulsion will be increased inasmuch as the specific gravity of the dispersing phase will approach more 70 nearly that of the continuous phase of the second emulsion.

I claim as my invention:

1. A fuel suitable for use in internal combustion engines comprising an emulsion of 75 hydrocarbon oil and water, cut back with hydrocarbon oil containing an oil soluble emulsifying agent capable of being expelled from the engine without substantial residue, the initial emulsion being in the dispersed 80 phase and the oil in the continuous phase.

2. A fuel suitable for internal combustion engines consisting of an initial emulsion of a relatively heavy gravity normally liquid hydrocarbon dispersed in water with a combustible emulsifying agent the water comprising the continuous phase of the initial emulsion, said emulsion being mixed in a lighter gravity liquid hydrocarbon with an emulsifying agent to form a final emulsion, 90 the lighter hydrocarbon comprising the continuous phase of the final emulsion, and the primary emulsion comprising the dispersed phase of the final emulsion.

3. A fuel suitable for internal combustion 95 engines consisting of a hydrocarbon oil emulsified with naphthenic acid in water, the water comprising the dispersed phase of the emulsion, said emulsion further diluted with hydrocarbon oil to predetermined 100 proportions of oil and water.

LESTER KIRSCHBRAUN.